

# UNITED STATES PATENT OFFICE.

HAROLD HIBBERT, OF PITTSBURGH, PENNSYLVANIA.

## MANUFACTURE OF EXPLOSIVES.

1,213,367.

Specification of Letters Patent. Patented Jan. 23, 1917.

No Drawing.

Application filed February 23, 1915. Serial No. 9,774.

*To all whom it may concern:*

Be it known that I, HAROLD HIBBERT, a subject of Great Britain, residing in Pittsburgh, Allegheny county, State of Pennsylvania, have invented certain new and useful 5 Improvements in the Manufacture of Explosives; and I do hereby declare the following to be a full, clear, and exact description of the invention, such as will enable others 10 skilled in the art to which it appertains to make and use the same.

The present invention is based upon the discovery that an explosive which will remain liquid at a temperature much below 15 that at which nitro-glycerin freezes can be produced by the nitrification of a mixture of glycols obtained primarily from the raw material known commercially as "oil gas"; and that, further, the mixture of glycols thus obtained can be added to glycerin and nitrated 20 simultaneously therewith, without other precautions than are customary in the manufacture of nitro-glycerin, and with the production of a product consisting in part of nitro-glycerin and in part of nitro-glycols, and 25 which partakes of the same quality of remaining unfrozen at relatively low temperatures.

A particular merit of the mixture of nitrated glycols obtained from oil gas, in accordance with the invention is that the mixture is relatively non-volatile, and is therefore capable of being used commercially under conditions which would be impracticable for some of its constituent nitrated glycols, as, for instance, nitrated butylene glycol which is too volatile to be used alone or to be incorporated with nitro-glycerin in the manufacture of blasting explosives.

40 In the practice of the invention, the primary "raw material" employed is oil gas, that is to say, gas obtained from the vaporization and gasification of a hydrocarbon oil, such as naphtha, solar oil, or the like. This 45 oil gas is subjected to a temperature within the range of 600° C.-900° C., in any suitable apparatus and is thereby cracked up into a mixture consisting essentially of about 50%-60% of unsaturated ethylene derivatives, the remainder consisting essentially of hydrogen, methane and ethane. The unsaturated derivatives referred to consist essentially of a mixture of ethylene, propylene and butylene, the proportions of these several constituents varying to some extent, ac-

cording to the apparatus employed, the temperature within the range stated, and the mode of heating. The mixture of unsaturated derivatives is then brought into contact with chlorin gas thereby forming the corresponding dichlor saturated derivatives and I thereupon saponify these chlorin compounds by heating them in the presence of an aqueous alkali carbonate solution at a temperature between 150° C.-200° C. in an apparatus capable of withstanding a considerable pressure.

The alkali carbonate solution that I prefer for the purpose is an aqueous solution of sodium carbonate, and I find that under the conditions specified an excellent yield of the corresponding glycols may be readily obtained by its use. The mixed glycol intermediate product thus obtained consists of a mixture of ethylene, propylene and butylene glycols. On subjecting the mixed glycol product to the action of a mixture of sulfuric and nitric acids, such as are used for the manufacture of nitro-glycerin, there is produced a mixture of nitrated glycols representing a very stable product and one capable of being used either wholly or in part as a substitute for nitro-glycerin in explosives.

Inasmuch as the hydrocarbons from which the glycols are produced are unsaturated hydrocarbons, the chlorin derivatives, and also the glycols themselves, will contain their respective chlorin or hydroxyl groups on adjoining atoms. Thus, for example, the 1-butylene, which is a constituent of the oil gas, will yield a glycol having the hydroxyl groups in 1.2 position. The isomeric 2-butylene will give the corresponding 2.3 glycol. The 1-butylene, however, usually predominates. Both glycols differ from the 1.3 glycols referred to in my prior Patents Nos. 994,841 and 994,842. The nitroglycols of the present invention are accordingly distinguished from the nitroglycols of said prior patents in that they contain the nitro groups on adjacent carbon atoms. The glycols used in the present invention are more stable in character, less volatile, and more easily nitrated.

As hereinbefore indicated, the nitrated product obtained from butylene glycol alone is too volatile to permit of its commercial utilization, either *per se*, or for incorporation with nitro-glycerin in the manufacture

of blasting explosives. On the other hand, the nitrated mixed glycol product obtained by the present invention represents a much less volatile product and one which may be used commercially as an explosive either with or without being incorporated with nitro-glycerin.

More particularly, the mixture of glycols may be mixed with glycerin, and the mixed product nitrated in the usual manner without the necessity of any precautions other than those usually adopted in the manufacture of nitro-glycerin, and with the great technical characteristic advantage that the mixed nitrated product has a very much lower freezing point than in the case of nitro-glycerin alone.

What I claim is:

1. An explosive comprising a nitrated mixture of glycols substituted on adjacent carbon atoms, said explosive being a stable product of a relatively non-volatile nature and of low freezing point; substantially as described.

2. An explosive comprising a mixture of nitrated glycols substituted on adjacent carbon atoms with other explosive compounds, said explosive being a stable product of a relatively non-volatile nature and of low freezing point; substantially as described.

3. An explosive comprising a mixture of nitrated glycols substituted on adjacent carbon atoms and glycerin, said explosive being a stable product of a relatively non-vol-

atile nature and of low freezing point; substantially as described. 35

4. An explosive comprising a nitrated mixture of ethylene, propylene and butylene glycols, said explosive being a stable product of a relatively non-volatile nature 40 and of low freezing point; substantially as described.

5. An explosive comprising a nitrated mixture of ethylene, propylene and butylene glycols with other explosive compounds, said explosive being a stable product of a relatively non-volatile nature and of low freezing point; substantially as described. 45

6. An explosive comprising a mixture 50 of nitrated ethylene, propylene and butylene glycols and nitrated glycerin, said explosive being a stable product of a relatively non-volatile nature and of low freezing point; substantially as described. 55

7. An explosive comprising a mixture of nitrated glycols one of which is nitrated butylene glycol substituted on adjacent carbon atoms, said explosive being a stable product of a relatively non-volatile nature 60 and of low freezing point; substantially as described.

In testimony whereof I affix my signature, in presence of two witnesses.

HAROLD HIBBERT.

Witnesses:

GEO. B. NICKEL,  
FRANK J. DAVIES.